

# United States Patent Office

2,834,076

Patented May 13, 1958

1

2,834,076

## HOT SAND CURING OF SHELL MOLDS

Julius M. Bleuenstein, Detroit, Mich., assignor to Ford Motor Company, Dearborn, Mich., a corporation of Delaware

No Drawing. Application August 12, 1953  
Serial No. 373,919

2 Claims. (Cl. 22—193)

This invention relates to the founding art and disclosures particularly an improvement in the currently utilized methods of preparing shell molds. Due to the fact that patterns for the formation of shell molds must withstand temperatures in excess of 350° F., they are invariably made of metal. To prepare a shell mold upon such a pattern it is conventional to secure the heated metal pattern to the open upper face of a sand box containing a mixture of molding sand of about No. 90 A. F. S. size containing about 7 percent of a heat settable phenol aldehyde resin. This assemblage of box and pattern is then inverted so that the heated pattern becomes the bottom of the box and the molding sand is dropped upon the hot pattern. This circumstance is allowed to continue for a period of time ranging up to 1 minute during which time a layer of the sand resin mixture immediately adjacent the heated pattern softens, partially cures and adheres to the heated pattern to form the shell. The heated pattern containing the attached shell is disengaged from the sand box and carried through an oven wherein it is exposed to radiant heat or direct flame to complete the curing of the resin and impart to the mold physical strength.

The instant invention utilizes the same procedure up to the curing step in the oven. Instead of curing the green mold in an oven, the metal pattern with the attached partly cured mold is again made the upper side of a second open topped sand box. However, this second sand box is filled with ordinary sand unmixed with resin but instead heated to a temperature between 350° F. and 1,300° F. After the pattern and mold have been secured to the top of this second box, the assemblage is inverted and permitted to remain in this position until the cure has been completed by virtue of the heat resident in the hot sand. This sand has been previously heated by direct fire located under the box when it is in the upright position in contradistinction to the inverted position.

It has been found that with an ordinary shell about  $\frac{1}{8}$  inch thick and with sand at 900° F. a complete cure may be effected in 15 seconds. This is more rapidly than can be done with radiant heat or direct flame and results in a mold which is more uniformly cured and hence has higher physical properties.

2

While ordinary sand has been disclosed as the heat carrying medium and has the advantages of not contaminating molds and being readily available, it is to be understood that any thermally stable pulverulent or granular material may be used. Experiments, for example, with iron shot have shown this material to be even faster than sand of the same temperature but it has the disadvantage of adhering to the mold. Other materials, such as suitably sized rock particles or iron oxide may obviously be employed as justified by special circumstances.

In the above description where the word mold is used, it is understood that the term is employed to include cores as well as molds.

15 I claim as my invention:

1. The process of preparing shell molds comprising heating a pattern, securing the heated pattern to an open topped sand box containing a mixture of sand and a heat settable resin, inverting the assemblage of sand box and pattern to shower the sand resin mixture upon the heated pattern, permitting the sand box to remain inverted until a shell of the desired thickness has been secured, detaching the pattern, carrying the shell from this sand box and attaching it to the top of a second open topped sand box containing sand heated to a temperature of 350° F. to 1,300° F., inverting the assemblage of the second sand box and pattern until the desired degree of cure of the resin is obtained, detaching the pattern from the second sand box and removing the shell.

2. The process of preparing shell molds comprising heating a pattern, securing the heated pattern to an open topped sand box containing a mixture of sand and a heat settable resin, inverting the assemblage of sand box and pattern to shower the sand resin mixture upon the heated pattern, permitting the sand box to remain inverted until a shell of the desired thickness has been secured, detaching the pattern, carrying the shell from this sand box and attaching it to the top of a second open topped sand box containing sand heated to a temperature of 350° F. to 1,300° F., inverting the assemblage of the second sand box and pattern until the desired degree of cure of the resin is obtained, detaching the pattern from the second sand box and removing the shell, said second box being heated while in the upright position by direct flame.

## References Cited in the file of this patent

### UNITED STATES PATENTS

|    |           |           |               |
|----|-----------|-----------|---------------|
| 50 | 414,122   | Roberts   | Oct. 29, 1889 |
|    | 489,194   | Mustin    | Jan. 3, 1893  |
|    | 2,493,498 | Peery     | Jan. 3, 1950  |
|    | 2,509,866 | Hemminger | May 30, 1950  |
| 55 | 2,670,573 | Sullivan  | Mar. 2, 1954  |

## OTHER REFERENCES

FIAT Final Report No. 1168, PB 81284, May 30, 1947.